

Patented Sept. 3, 1929.

1,727,180

# UNITED STATES PATENT OFFICE.

BY RAMJI D. SAKLATWALLA, OF CRAFTON, PENNSYLVANIA, ASSIGNOR TO VANADIUM CORPORATION OF AMERICA, OF BRIDGEVILLE, PENNSYLVANIA, A CORPORATION OF DELAWARE.

## VANADIUM-ALUMINUM-SILICON ALLOY.

No Drawing.

Application filed February 2, 1928. Serial No. 251,467.

This invention relates to a composition of alloy containing vanadium as the major constituent, together with aluminum and silicon, and containing negligible percentages of carbon.

In the manufacture of vanadium steel in the basic open hearth process, the vanadium, usually in the form of ferro-vanadium, is added to the molten steel after it has been tapped into the ladle. If the vanadium were added to the steel bath in such a basic furnace instead of in the ladle there would be considerable loss of vanadium, owing to the oxidizing conditions existing in the furnace.

In the acid open hearth or the electric furnace process vanadium is added in the furnace, although part of the vanadium, especially material in finely divided state, is generally added in the ladle. It is well-known in steel making practice that the less the total amount of cold material added in the ladle the better and more uniform are the ingots obtained from pouring such steel. The cold material introduced into the ladle absorbs heat in the process of melting and dissolving in the molten bath and consequently reduces the ladle temperature, thus creating the danger of pouring the steel into the molds at a lower temperature than that

requisite for the production of sound ingots. Also, if the steel tapped into the ladle is not completely deoxidized, the oxides present therein will effectually burn up some of the vanadium content of the ferro-vanadium added. To offset this deficiency, the steel is deoxidized prior to addition of ferro-vanadium by means of silicon metal or alloys, or aluminum, or both. By the process of my invention, I propose to incorporate the deoxidizing agents, like aluminum and silicon, into the body of the vanadium alloy, whereby the deoxidation procedure will proceed simultaneously with the alloying of the vanadium into the steel. By combining the silicon and aluminum with the vanadium in the alloy, very much less material is added into the ladle, inasmuch as the cold iron which would be added in combination with the vanadium and the silicon separately, as ferro-vanadium and ferro-silicon, would be very much greater than the iron present in the composition of my invention. Besides the decrement of temperature produced by the addition of inert cold iron, the disadvantage was always present that unnecessary percentages of other

impurities, such as sulphur and phosphorus, were introduced into the molten steel, such impurities being proportionate to the amount of cold iron present and being derived from the scrap iron used in the manufacture of the separate ferro alloys. If, therefore, two or three separate alloys were added, each with the same percentages of objectionable impurities as in the alloy of my invention, it is easy to see that the impurities in the steel will accumulate to two or three fold extent. It is also well-known that ferro alloys containing high percentages of silicon and aluminum show a very much less carbon content and prevent the formation of carbides than if this silicon and aluminum content were absent. A vanadium alloy therefore containing percentages of aluminum and silicon incorporated in the alloy will carry correspondingly less carbides.

Moreover, the vanadium content of the alloy will be protected against loss by oxidation by the aluminum and silicon present, since the aluminum and silicon are more readily oxidizable than the vanadium.

A vanadium alloy containing aluminum and silicon can be produced with practically negligible quantities of iron, so that such an alloy can be utilized for introducing vanadium into non-ferrous metals such as the various aluminum alloys and bronzes. It can also be used in other non-ferrous metals where the presence of iron would be detrimental but that of silicon or aluminum would not be objectionable.

I obviate the deficiencies enumerated above by producing an alloy containing vanadium from 40% to 90%, preferably from 70% to 90%, together with aluminum from 3% to 15%, and silicon from 5% to 30%, the carbon content of the alloy being negligible, approximately under .50%. The vanadium, aluminum, and silicon contents of the alloy can be varied to suit the particular specifications of the finished steel to which these alloys have to be added. As examples of typical compositions I give the following:

- (1) Vanadium, approximately 40%.  
Aluminum, approximately 8%.  
Silicon, approximately 16%.  
Iron, approximately 36%. 105
- (2) Vanadium, approximately 62½%.  
Aluminum, approximately 12½%.  
Silicon, approximately 25%.  
Iron, negligible. 110

- (3) Vanadium, approximately 82%.  
 Aluminum, approximately 6%.  
 Silicon, approximately 12%.  
 Iron, negligible.
- 5 (4) Vanadium, approximately 88%.  
 Aluminum, approximately 4%.  
 Silicon, approximately 8%.  
 Iron, negligible.

An alloy containing the high percentages 10 of vanadium, together with the silicon and aluminum contents, and low in iron content, together with absence of carbides, is very readily soluble in molten steel, much more so than the alloys containing low percentages 15 of vanadium and of such other characteristics as are found on the market today. Further, since such alloys have the deoxidizing reagents combined in them, they will produce a cleansing of the steel at the moment of its 20 alloying with vanadium, so that the diffusion of the alloying element in such steel will be more complete, producing more homogeneous ingots. Also, there will be an assurance of the vanadium not being utilized for the 25 purpose of combining with the oxides present in the steel and thus being lost in the slag, but will effectually and completely enter into the steel, the removal of the dissolved oxides being accomplished by the aluminum and the 30 silicon. Further, since the aluminum content in these alloys is always accompanied by a silicon content, the product of oxidation will not be an infusible alumina, which, as is well known, remains disseminated in the steel 35 upon its solidification, but will be a fusible low melting aluminum silicate which will rise through the molten steel and be eliminated.

The alloy of my invention, containing approximately from 40% to 90% vanadium, 40 from 3% to 15% aluminum, and from 5% to 30% silicon, with less than .50% carbon, can be produced in the electric furnace by the use of a suitable reducing agent, such as silicon. However, I prefer to obtain the reduction of the vanadium content from a very 45 high grade of vanadium pentoxide by means of aluminum as the reducing agent, according to the well-known process of aluminothermic reduction. The advantage of the 50 alumino-thermic reduction is the facility of obtaining these alloys with practically no carbon contamination, which is more difficult to achieve in an electric furnace reduction.

While I have described my alloy in its 55 preferred composition, it is to be understood that the invention is not so limited but may be otherwise embodied within the scope of the following claims.

I claim:

1. A vanadium alloy containing about 40% 60 to 90% vanadium, about 3% to 15% aluminum, and about 5% to 30% silicon, the remainder being principally iron.

2. A vanadium alloy containing about 40% 65 to 90% vanadium, about 3% to 15% aluminum, and about 5% to 30% silicon, and containing less than .5% carbon, the remainder principally iron.

3. A vanadium alloy substantially free 70 from iron and containing aluminum and silicon as its alloying elements, the vanadium content being over 40%, and containing less than .5% carbon.

4. A vanadium alloy containing about 70% 75 to 90% vanadium, about 3% to 15% aluminum, about 5% to 25% silicon, and containing less than .5% carbon, the remainder being principally iron.

5. The process of treating a bath of molten metal, which comprises adding to such metal 80 a vanadium alloy containing aluminum and silicon, thereby deoxidizing the bath by means of the aluminum and silicon simultaneously with the process of alloying the vanadium with the bath metal, and forming 85 an easily fusible aluminum silicate slag.

6. The process of making a vanadium containing steel, which comprises adding to a bath of the molten steel a vanadium alloy containing aluminum and silicon as deoxidizing agents, whereby the steel is deoxidized 90 simultaneously with the addition of the alloying vanadium, and a low melting point aluminum silicate slag is formed.

7. An alloy substantially free from iron 95 and containing vanadium, aluminum and silicon as essential elements, the percentage of vanadium being greater than the aluminum or silicon, and containing less than .50% carbon.

8. An alloy containing vanadium, aluminum and silicon as essential elements and together constituting the greater part of the alloy, the vanadium being greater in amount than either the aluminum or the silicon, the remainder of the alloy being principally iron.

9. An alloy containing vanadium as its major constituent together with smaller but effective amounts of both aluminum and silicon.

10. An alloy containing vanadium as its major constituent together with smaller but effective amounts of both aluminum and silicon, and containing less than .5% carbon.

In testimony whereof I have hereunto set my hand.

BYRAMJI D. SAKLATWALLA.